

## UNITED STATES PATENT OFFICE

JAMES A. CARSON, OF SALT LAKE CITY, UTAH, ASSIGNOR TO UTAH METALS FLUX COMPANY, OF SALT LAKE CITY, UTAH, A CORPORATION OF UTAH

## PROCESS OF MAKING IRON AND STEEL AND PRODUCT

No Drawing.

Application filed March 4, 1930. Serial No. 433,188.

This invention relates to the production of iron directly from its ore having remarkable properties as compared with cast iron and in many respects equal to or better than the properties of ordinary carbon steels.

A suitable procedure in accordance with my invention is as follows:

40 pounds of 50 per cent iron oxide ore, such as that found in the iron ore deposits 10 in Michigan, and 6 pounds of shale, such as that found in the northern central portion of Emery County, Utah, southeast of Price, Utah, and south of Price River and Desert 15 Lake, are placed in a crucible in alternate layers beginning with the shale at the bottom and heated to about from 2900 to 3200° F. for about 3 to 3½ hours. The mass boils during the heating thereby providing its own agitation. The metal is then poured 20 into a billet, for instance in an iron mold, allowed to cool until it has solidified then broken out of the mold and allowed to cool on the floor. In this form and without any further treatment it has a carbon content 25 of about 1.02%, a Brinnell hardness of 304, is very tough but easily machined and shows a fine, close fibrous grain. It takes a high polish, is highly resistant to corrosion and to the action of the weaker acids, and can 30 be tempered by the methods customarily employed for treating carbon steels.

A satisfactory chemical analysis of the shale used in this process cannot be given, but the shale may be further described and 35 identified as varying in color from light yellow to dark brown, having a silky texture and a greasy feel, and containing dikes or veins or impregnations of a material of jet black color. It is found associated with 40 the so-called Dakota sand stone deposits. Two particular deposits of the shale are located at Township-Range 17 South, 10 East, Sections 12 and 24.

I have further found that the metal produced as described above or even cast iron, which has been treated as described in United States Letters Patent No. 1,712,879 dated May 14, 1929, to Ernest S. Fisher, with the shale above referred to, that is, 45 by cooking the metal with 1 to 10%, pref-

erably 4 to 6% of the shale, when melted together with about an equal weight of ordinary scrap steel gives, upon casting, a metal of light gray color having a close granular grain, capable of taking a high 55 polish and having a Brinnell hardness of about 220, and a tensile strength of from 30,000 to 36,000 pounds per square inch. This metal is easily poured into fine close grained castings free from pin holes and 60 pits, and can be poured under ordinary casting conditions at much lower temperatures than ordinary cast iron. It is easily machined and can be heat-treated at 1200° F. and cold-quenched to a product suitable 65 for use as die rings, etc. It resists corrosion better than ordinary cast iron. A typical analysis shows 2.35% silicon and 3.4% carbon and a very low sulfur and phosphorus content.

70 My invention is not limited specifically to the details of procedure described, excepting as may be required by the terms of the appended claims. The proportion of ore to shale, the specific manner of heating them 75 in contact with each other, the temperature and time of heating, all may be varied and other materials may be added to the mixture.

## I claim:

1. Process which comprises heating a mixture of iron oxide ore and shale substantially identical with that found in the northern central portion of Emery County, Utah, south of Price River and Desert Lake, to a temperature of about from 2900 to 3200° 80 F. and casting the resulting metal.

2. Process which comprises heating a mixture of about 40 parts by weight of 50 percent iron oxide ore and 6 parts by weight of shale substantially identical with that 85 found in the northern central portion of Emery County, Utah, south of Price River and Desert Lake, to a temperature in the neighborhood of 3000° F. for about 3 hours and casting the resulting metal.

3. As a new product, cast metal produced by heating iron oxide ore with shale substantially identical with that found in the northern central portion of Emery County, Utah, south of Price River and Desert Lake,

to a temperature in the neighborhood of 3000° F., and casting the resulting metal, said product consisting principally of iron and having a carbon content of about 1% and being capable of being tempered by the methods customarily employed for treating carbon steel.

In testimony whereof, I affix my signature.  
**JAMES A. CARSON.**

**10****15****20****25****30****35****40****45****50****55****60****65**